

# UNITED STATES PATENT OFFICE.

SOPHIA E. SCHUER, OF WARREN, MICHIGAN.

## IMPRESSION-PAPER.

1,377,368.

Specification of Letters Patent. Patented May 10, 1921.

No Drawing.

Application filed April 21, 1919. Serial No. 291,568.

To all whom it may concern:

Be it known that I, SOPHIA E. SCHUER, a citizen of the United States of America, residing at Warren, in the county of Macomb 5 and State of Michigan, have invented certain new and useful Improvements in Impression-Paper, of which the following is a specification.

This invention relates to the manufacture 10 of a coated paper particularly adapted for artist's use in tracing the outlines of drawings and the like, which is commonly used by placing it between the drawing to be copied and a sheet to receive the impression, 15 with the coated side of the paper against the impression receiving sheet, and it is therefore of importance that the coating be such that it will be readily impressed upon the receiving sheet, leaving clear, clean lines 20 without smutting, and that the composition of the coating be such that the impressed lines may be readily erased from the receiving sheet if desired. Further, it is necessary that the composition of material forming 25 the coating be such that the lines impressed may be worked over with ink, water colors, paints or other material used by artists, and such that the coating will not readily rub off in handling.

30 The object of the invention is to provide a coated paper or a coating material for paper having the above and other desirable characteristics, the invention consisting in the matters hereinafter set forth and more particularly pointed out in the appended claims.

The coating material consists of soft soap made in the usual manner by boiling fatty substances with a lye usually derived from wood ashes, or potash, thus decomposing the 40 fats into acids and then incorporating therewith a sufficient quantity of fine carbon material, such as a soot deposit from the smoke of burning soft coal, to make a thin black paste. This paste is then spread, in any 45 suitable manner, upon sheets, preferably of thin paper and allowed to dry. It may then be burnished or given a smooth glossy finish by passing any suitable device having a smooth hard surface, over the surface of the 50 coating.

A paper particularly adaptable for artist's use in tracing is thus provided, the coating lying wholly upon the surface of the paper but adhering firmly thereto, and having sufficient hardness so that it will not rub off too freely and smut the fingers, paper, or other things with which it comes in contact, while at the same time leaving a clear black line impression in tracing without requirement of undue pressure of the tracing instrument 55 thereon. The coating being free of oily or greasy substances, does not penetrate the paper with which it is coated and will not soil the impression sheet or interfere with the working over of the lines impressed 60 thereon, with ink, water colors, or any other of the materials used by artists in making pictures. Further, the impressed lines may be as readily and cleanly erased as lead pencil marks, due to non-penetration of the substance forming the coating and the absence 70 of free oil or grease, and this coated paper does not deteriorate with age.

The composition of material permits of giving the coating a glossy finish by simply 75 smoothing the surface by frictional contact of a hard smooth surface therewith, thus making the material less liable to rub off and giving an attractive appearance.

The preparing and applying of the coating 80 may be carried out by hand or by suitable machinery as desired, and a very efficient and durable paper which is cheap to manufacture is secured.

Having thus fully described my invention 85 what I claim is:—

1. An impression paper comprising a carrying sheet coated with a composition of soft soap and soft coal soot.
2. An impression paper comprising a carrying sheet and a coating on said sheet consisting of a soft soap, and soft coal soot, the coating being free from grease or soluble coloring matter.

In testimony whereof I affix my signature 95 in the presence of two witnesses.

SOPHIA E. SCHUER.

Witnesses:

ANNA M. DORR,  
LEWIS E. FLANDERS.